

April 29, 1930.

O. E. BUCKLEY  
ELECTRICAL CONDUCTOR

1,756,341

Filed Dec. 31, 1924

Fig. 1



Fig. 2



Fig. 3



Inventor:  
Oliver E. Buckley,  
by Edward A. Atty

## UNITED STATES PATENT OFFICE

OLIVER E. BUCKLEY, OF MAPLEWOOD, NEW JERSEY, ASSIGNOR TO WESTERN ELECTRIC COMPANY, INCORPORATED, OF NEW YORK, N. Y., A CORPORATION OF NEW YORK

## ELECTRICAL CONDUCTOR

Application filed December 31, 1924. Serial No. 758,984.

This invention relates to conductors for the transmission of electrical energy and more particularly to signaling conductors having an external layer of a material of high permeability for the purpose of increasing the inductance of the conductor.

One manner of increasing the inductance of the conductor employed for the transmission of alternating current is to wrap the conductor spirally with a layer of wire or tape of magnetic material. This method is known in the art as continuous inductive loading as distinguished from lump loading by means of inductance coils distributed at intervals along the conductor. Until recently iron has been considered to be the only material suitable for continuous loading but it has now been discovered that a more suitable material may be procured in the form of an alloy of nickel and iron. When these two metals are combined in the proper proportions and the resulting alloy is given a proper heat treatment, a material having a very high permeability at low magnetizing forces is obtained.

One form of this material which has been used in a submarine cable comprises 78½% nickel and 21½% iron. Alloys of nickel and iron having similar characteristics, especially high permeability at low magnetizing forces have been styled "permalloy." Other properties possessed by these alloys which increase their value as a loading material are a hysteresis loss lower than that of iron and a high resistivity, both properties being conducive to increasing the efficiency of the cable by lowering the effective resistance of the conductor. When it was attempted to employ this material in the form of a tape for continuous loading, difficulties were encountered. It was found that if the permalloy tape was first heated and then cooled before applying to the conductor, internal stresses were set up upon bending of the tape, causing the permeability to be very materially lowered. This difficulty was overcome by applying the tape to the con-

ductor before giving the tape the heat treatment and then subjecting the taped conductor to the heating and cooling necessary to produce high permeability in the loading material.

Further difficulty, however, was experienced in that the permeability of the loading material was lowered by what appeared to be adhesion between the copper conductor and the loading tape. It is believed that this adhesion occurs when the taped conductor is subjected to the high temperatures necessary for the proper heat treatment and that upon subsequent cooling the tape is subjected to stresses which cause a lowering of its permeability.

In the construction of a loaded conductor it was the practice to wrap a layer of magnetic material comprising a nickel-iron alloy closely around the conductor consisting of a central copper wire surrounded by six flat copper strands, the whole making a compact structure with very little space not occupied by metal. To give the loading material the desired magnetic characteristics, this conductor was heated to approximately 850° C. and then cooled at a preferred rate. On heating, both metals expand but the copper, because of its higher temperature coefficient, expands more than the loading material with the result that it presses tightly against the loading material when the conductor is at the high temperature and if the structure is a fairly tight one, the magnetic tape is stretched, an elongation of 1% having been observed. This stretching has apparently no direct effect on the magnetic properties since it occurs at a temperature above the magnetic transformation point but it does show effects of high pressure between the metals. At the temperature of 850° C. both metals are relatively soft and since they are forced together by thermal expansion there is a tendency for the loading material to weld to the copper, the extent to which the metals are welded depend-

ing on several factors such as the tightness of the copper structure and the character of the metal surfaces. In this connection it has been noted that although the loading material welds to the copper, welding of the copper strands to the central wire has been very rarely observed and no welding has been observed between layers of the loading material when more than one layer has been used. 10 These results suggest that welding is possibly not a simple case of fusion of the two metals but some effect brought about by chemical action.

On cooling, the copper conductor contracts 15 more than the magnetic tape. No doubt some of the welds which have been formed break loose when this contraction occurs but the stronger ones hold with the result that the magnetic tape is at points pulled down with 20 the copper and parts of it are bent, stretched or compressed depending upon the particular accidental conditions of adherence. Even though the forces involved may be very small, the stresses at points in the tape may be of 25 considerable magnitude giving strain sufficient to reduce the permeability at spots to a very small fraction of that which the tape would have had if not subjected to such strain. The resultant conductor, therefore, is one 30 which although it may have fairly uniform inductance as measured from foot to foot is loaded with a material which varies in permeability over a wide range in points separated by a fraction of an inch.

35 The copper strands upon being stranded about the central conductor do not present a true cylindrical surface since the edges of the strands do not lie in close contact with the central conductor but present spiralled edges. 40 As the cooling proceeds, therefore a sticking or welding of the material may occur at various points along these edges and the subsequent contraction of the copper set up stresses in the alloy tape.

45 During the cooling portion of the heat treatment the alloy tape may cool more rapidly at first than does the copper conductor due to its intimate contact with the cooling medium so that the alloy tape quickly comes into intimate contact with the copper strands.

Whatever may be the true explanation for the difficulty experienced, it has largely been overcome by providing a small air space between the layer of loading material and the 55 signaling conductor when the loading material is applied. This method of obtaining high permeability is described at length in patent to G. W. Elmen, No. 1,586,887, issued on June 1, 1926.

60 Instead of providing an air space between the conductor and the tape, as the latter is wound in position, the desired result may be obtained by placing a layer of paper upon the conductor before the loading material is 65 wound thereon. This layer of paper is

burned out during the subsequent heat treatment thus giving the desired spacing between the loading material and the conductor. This method is described in detail in patent to W. B. Ten Eyck No. 1,586,862, issued on June 1, 1926. 70

During the heat treatment the loaded conductor is passed through a heated tube for the purpose of securing the desired permeability of the loading tape. It has been found that if any grease, oil, or carbonaceous material is, by accident or otherwise, attached to the heating chamber or the conductor as it passes through the heating chamber reducing gases such as hydrogen or carbon monoxide are released. All copper wire of high conductivity which it is possible to obtain on the open market contains a certain amount of copper oxide, and when the copper conductor is heated in the presence of a reducing atmosphere, the copper oxide is dissolved, thereby rendering the conductor brittle. Various means have been proposed for preventing this embrittling action, such for example, as the method disclosed in patent to J. W. Harris No. 1,586,897, issued on June 1, 1926. In this method, which has been the preferred method used commercially heretofore, a stream of nitrogen is forced through the heating tube in a direction opposite to the direction of movement of the conductor, thereby sweeping out the reducing gases as soon as they are released and thus protecting the conductor. This process, however, is expensive, and moreover, is objectionable because of the fact that there is always an element of risk involved since failure of the flow of nitrogen might be of serious consequence. 90

An object of the present invention is to provide for the practical loading of a signaling conductor with magnetic material which requires heat treatment and whose characteristics are subject to undesired change under applied stresses. 105

Another object of the invention is to provide a method of applying magnetic loading material to an electrical conductor in such a manner as to prevent the setting up of deleterious stresses in the magnetic material during the subsequent heat treatment. 110

A further object of the invention is to subject the loaded conductor to the desired heat treatment without danger of embrittling the conductor. 115

To accomplish these objects, the invention contemplates an electrical conductor upon which is applied a loading material capable of possessing high permeability and the method of applying this material to the conductor in such a way as to avoid obtaining low or variable values of permeability. This invention is in the nature of an alternative to those disclosed in the above mentioned patents to G. W. Elmen and W. B. Ten Eyck. Each of these inventions has certain advan- 120 125

tages over the others as will be apparent from a consideration of the several patents.

The invention may be more clearly understood by reference to the accompanying drawing in which—

Fig. 1 is a view of a loaded conductor, certain portions being shown cut away to more clearly disclose the structure;

Fig. 2 is a cross-sectional view of the conductor of Fig. 1; and

Fig. 3 is a view showing apparatus which may be used for applying the heat treatment to the conductor.

Referring to the drawing, the electrical conductor preferably comprises a central core member 10 of conducting material about which a plurality of conducting strands 11—11 are wrapped with a spiral lay. About this composite conductor is wrapped the tape 12 which preferably consists of an alloy containing 78½% nickel and 21½% iron. The surfaces of member 10 and strands 11—11 are provided with a coating of copper oxide, which preferably is formed at the time of annealing the individual parts of the composite conductor. This may be accomplished by simply exposing the copper conducting strands to air at a suitable stage in the annealing process instead of protecting them from air during annealing as is ordinarily done in commercial practice.

After the stranded conductor is formed of the central oxidized copper wire and the oxidized copper tape and the composite conductor is provided with one or more layers of permalloy tape applied sufficiently tightly to make a good mechanical structure, the resulting conductor is treated by passing it through a heated tubular furnace of the type disclosed in Fig. 3. This furnace which is of the muffle type comprises heating elements 30 which are located between the fire clay muffle 31 and the fire brick 32. The iron tube 33 has a copper lining 34 of such small inside diameter as to prevent rapid circulation of air which would cause an objectionable degree of oxidization of the permalloy tape. For the sake of clearness this apparatus has been shown schematically but reference is made to an application of F. S. Kochendorfer, Serial No. 601,921, filed November 15, 1922, which has issued as Patent No. 1,624,668 on April 12, 1927 and which discloses the preferred form of apparatus to be used.

With a structure constructed as described danger of embrittling the conductor during the heat treatment is eliminated, even though grease, oil or other matter is attached to the conductor as it enters the furnace and even though this foreign matter produces reducing gases, since these gases will first attack the copper oxide on the surface of the copper and if this oxide is sufficient in amount no action will take place tending to embrittle the copper until the surface copper oxide has

first been reduced. It has been determined that a very thin layer of black copper oxide will be effective in preventing embrittling of the copper.

The coating of copper oxide furthermore prevents the copper conductor from alloying with the magnetic tape when the taped conductor is subjected to the high temperatures required for the heat treatment. Therefore, adhesion between the conductor and tape during the cooling process with resulting stresses in the material is prevented and the high permeability of the material is maintained.

While the use of a layer of metallic oxide between the conductor and loading material has been described as applied to a stranded conductor, its use is of particular importance in preventing adhesion when applied to a solid conductor. In the case of a loaded stranded conductor, there is a certain amount of looseness in the structure which prevents adhesion and which is not present when the loading tape is wound on a solid conductor. Therefore, in the latter case there is an even greater necessity for providing some means for preventing adhesion.

What is claimed is:

1. In a continuously loaded conductor which requires a heat treatment to high temperatures to develop one of its magnetic properties, a copper conductor having near its surface a zone of a material containing a far greater amount of oxygen per unit volume than does the conductor at its center.

2. A loaded signaling conductor comprising a central conductor, a coating of reducible material about said copper conductor, and a magnetic loading material forming a wrapping close about the coated conductor, said loading material when on said coated conductor requiring heating to high temperature to develop high permeability therein and the permeability of which is sensitive to strain.

3. A loaded signaling conductor comprising a central conductor, a coating of metallic oxide about said conductor, and a magnetic loading material forming a wrapping close about the coated conductor, said loading material after being placed on said coated conductor requiring heating to high temperature to develop high permeability therein and the permeability of which is sensitive to strain.

4. A loaded signaling conductor comprising a central copper conductor, a coating of metallic oxide about said conductor, and a magnetic loading material wrapped closely about the coated conductor, said loading material after being placed on said coated conductor requiring heating to high temperature to develop high permeability therein and the permeability of which is sensitive to strain.

5. A loaded signaling conductor comprising a central conductor, a coating of copper oxide about said copper conductor, and a magnetic loading material forming a wrapping close about the coated conductor, said 5 loading material being in such a state that it requires a heating and cooling treatment to develop high permeability therein and the permeability of which is sensitive to strain. 6. A loaded signaling conductor comprising 10 a central copper conductor, a coating of copper oxide about said conductor, and a magnetic loading material forming a wrapping close about the coated conductor, said loading material comprising a nickel iron 15 alloy consisting of approximately 78½% nickel and 21½% iron and being in such a magnetic state that it requires a heating and a cooling process to improve its permeability. 7. A method of continuously loading a 20 copper conductor with magnetic material which requires a heat treatment to high temperature after its application to the conductor in accordance with which a supply of metallic oxide is placed under the loading material before the commencement of said heat treatment, said supply being sufficient to materially reduce embrittlement of the copper due to the presence of reducing gases 25 during said heat treatment. 8. A loaded signaling conductor comprising a central copper conductor, a magnetic loading material to be heat treated after its application to the conductor composed largely 30 of nickel and iron and enveloping said conductor, and a spacer of copper oxide separating said conductor and said loading material to prevent interaction therebetween and to prevent embrittling of said conductor 35 during a heating process which may be applied to said loaded conductor to improve the permeability of said loading material. 9. The method of constructing a continuously loaded signaling conductor which 40 comprises treating the surface of the conductor to produce a layer of metallic oxide thereon, placing a layer of loading material over the metallic oxide and heat treating the loaded conductor. 45 10. The method of constructing a continuously loaded signaling conductor which comprises treating the surface of the conductor to provide a layer of copper oxide thereon, placing a layer of loading material 50 over the copper oxide and heat treating the loaded conductor. 55 11. The method of continuously loading a copper conductor which comprises producing a surface coating of copper oxide on the 60 conductor during the annealing process, covering the conductor with a loading material requiring heat treatment, and heat treating the loaded conductor. 65 12. The method of constructing a continuously loaded copper conductor which com- 70 75 80 85 90 95 100 105 110 115 120 125 130
- prises producing a surface coating of copper oxide on copper strands during the process of annealing, winding a plurality of said strands spirally about a central copper strand to form a composite stranded conductor, placing a layer of loading material requiring heat treatment over said stranded conductor, and heat treating the loaded conductor. In witness whereof, I hereunto subscribe my name this 26th day of December, A. D. 1924.
- OLIVER E. BUCKLEY.